



US008372242B2

(12) **United States Patent**  
**Ales et al.**

(10) **Patent No.:** **US 8,372,242 B2**  
(b5) **Date of Patent:** **Feb. 12, 2013**

(54) **CONDUCTIVE WEBS AND PROCESS FOR  
MAKING SAME**

(75) Inventors: **Thomas Michael Ales**, Neenah, WI (US); **Davis-Dang H. Nhan**, Appleton, WI (US); **Duane Joseph Shukoski**, Neenah, WI (US); **Michael John Rekoske**, Appleton, WI (US)

(73) Assignee: **Kimberly-Clark Worldwide, inc.**, Neenah, WI (US)

(\*) Notice: Subject to any disclaimer, the term of this patent is extended or adjusted under 35 U.S.C. 154(b) by 0 days.

(21) Appl. No.: **13/465,876**

(22) Filed: **May 7, 2012**

(65) **Prior Publication Data**

US 2012/0216973 A1 Aug. 30, 2012

**Related U.S. Application Data**

(63) Continuation of application No. 12/341,419, filed on Dec. 22, 2008, now Pat. No. 8,172,982.

(51) **Int. Cl.**

**D21H 13/50** (2006.01)  
**D21F 11/00** (2006.01)  
**B28B 21/48** (2006.01)

(52) **U.S. Cl.** ..... **162/145**; 162/118; 162/138; 162/120; 162/205; 162/164.1; 162/182; 162/183; 162/194; 83/56; 242/525; 242/530.4; 242/542

(58) **Field of Classification Search** ..... 162/118, 162/120, 122, 141, 145, 152, 158, 164.1, 162/168.1, 194, 204, 205, 182, 183; 83/13, 83/56; 242/520, 525.3, 530.1, 530.4, 542

See application file for complete search history.

(56)

**References Cited**

**U.S. PATENT DOCUMENTS**

|                |         |                         |           |
|----------------|---------|-------------------------|-----------|
| 1,347,872 A *  | 7/1920  | Pringle .....           | 242/525.1 |
| 2,256,082 A *  | 9/1941  | Feurt .....             | 242/521   |
| 3,348,477 A *  | 10/1967 | Taylor, Jr. et al. .... | 101/23    |
| 4,422,588 A *  | 12/1983 | Nowisch .....           | 242/524.1 |
| 4,508,282 A *  | 4/1985  | Eiting .....            | 242/419.4 |
| 4,695,006 A *  | 9/1987  | Pool .....              | 242/525.2 |
| 4,989,487 A *  | 2/1991  | Staley .....            | 83/506    |
| 5,017,268 A *  | 5/1991  | Clitherow et al. ....   | 162/146   |
| 5,193,423 A *  | 3/1993  | Bakker .....            | 83/24     |
| 6,129,304 A *  | 10/2000 | Biagiotti .....         | 242/530.1 |
| 6,183,601 B1 * | 2/2001  | Otto et al. ....        | 162/205   |
| 6,524,445 B1 * | 2/2003  | Otto et al. ....        | 162/361   |
| 6,561,064 B1 * | 5/2003  | Hada et al. ....        | 83/13     |
| 6,985,790 B2 * | 1/2006  | Begemann et al. ....    | 700/127   |
| 7,114,422 B1 * | 10/2006 | Neuland et al. ....     | 83/29     |

(Continued)

**FOREIGN PATENT DOCUMENTS**

WO WO 2010073133 A2 \* 7/2010

**OTHER PUBLICATIONS**

Machine Translation of JP 2002-266217, published on Sep. 18, 2002.\*

(Continued)

*Primary Examiner* — Jose A Fortuna

(74) *Attorney, Agent, or Firm* — Dority & Manning, P.A.

(57) **ABSTRACT**

Conductive nonwoven webs are disclosed. The nonwoven webs contain pulp fibers combined with conductive fibers. In one embodiment, the webs are made in a wetlaid tissue or paper making process. The pulp fibers contained in the webs may comprise softwood fibers, while the conductive fibers may comprise carbon fibers. Base webs can be produced having a resistance of less than about 100 Ohms/square in one embodiment. Once produced, the conductive material can be cut into slits that are then wound on spools. From the spools, the conductive slits can be fed into a process for making any suitable product.

**12 Claims, 10 Drawing Sheets**



**U.S. PATENT DOCUMENTS**

7,944,401 B2 \* 5/2011 Gakhar et al. .... 343/718  
8,025,764 B2 \* 9/2011 Bhat et al. .... 162/117  
8,058,194 B2 \* 11/2011 Nhan et al. .... 442/414  
8,172,982 B2 \* 5/2012 Ales et al. .... 162/145  
2006/0144543 A1 \* 7/2006 Aho et al. .... 162/164.6  
2006/0191656 A1 \* 8/2006 Buzzza et al. .... 162/158  
2006/0207735 A1 \* 9/2006 Blanz et al. .... 162/111  
2006/0207738 A1 \* 9/2006 Wild .... 162/168.1  
2009/0036012 A1 \* 2/2009 Nhan et al. .... 442/268  
2009/0036015 A1 \* 2/2009 Nhan et al. .... 442/335  
2009/0036850 A1 \* 2/2009 Nhan et al. .... 604/361  
2009/0176074 A1 \* 7/2009 Sotendahl et al. .... 428/208

2009/0294435 A1 \* 12/2009 Nhan et al. .... 219/553  
2009/0321238 A1 \* 12/2009 Nhan et al. .... 200/5 A  
2010/0155006 A1 \* 6/2010 Ales et al. .... 162/149  
2011/0108225 A1 \* 5/2011 Buzzza et al. .... 162/164.3  
2012/0055641 A1 \* 3/2012 Nhan et al. .... 162/125  
2012/0071362 A1 \* 3/2012 Nhan et al. .... 506/33  
2012/0216973 A1 \* 8/2012 Ales et al. .... 162/118

**OTHER PUBLICATIONS**

Machine Translation of JP 2004-342509, published on Dec. 2, 2004.\*

\* cited by examiner



FIG. 1



FIG. 2



FIG. 3



FIG. 4



FIG. 5



FIG. 6



FIG. 7



FIG. 8



FIG. 9



FIG. 10

## CONDUCTIVE WEBS AND PROCESS FOR MAKING SAME

### RELATED APPLICATIONS

The present application is a continuation application and claims priority to U.S. patent application Ser. No. 12/341,419, filed on Dec. 22, 2008, now U.S. Pat. No. 8,172,982, and which is incorporated herein by reference.

### BACKGROUND

Absorbent articles such as diapers, training pants, incontinence products, feminine hygiene products, swim undergarments, and the like conventionally include a liquid permeable body-side liner, a liquid impermeable outer cover, and an absorbent core. The absorbent core is typically located in between the outer cover and the liner for taking in and retaining liquids (e.g., urine) exuded by the wearer.

The absorbent core can be made of, for instance, superabsorbent particles. Many absorbent articles, especially those sold under the tradename HUGGIES™ by the Kimberly-Clark Corporation, are so efficient at absorbing liquids that it is sometimes difficult to tell whether or not the absorbent article has been insulted with a body fluid.

Accordingly, various types of moisture or wetness indicators have been suggested for use in absorbent articles. The wetness indicators may include alarm devices that are designed to assist parents or attendants identify a wet diaper condition early on. The devices can produce an audible signal.

In the past, for instance, wetness indicators have included an open circuit incorporated into the absorbent article that is attached to a power supply and an alarm device. When a conductive substance, such as urine, is detected in the absorbent article, the open circuit becomes closed causing the alarm device to activate. The open circuit may comprise, for instance, two conductive elements that may be made from a metal wire or foil.

Problems have been experienced, however, in efficiently and reliably incorporating wetness indicators into absorbent articles at the process speeds at which absorbent articles are produced. Thus, a need exists for improved wetness sensors that can be easily incorporated into absorbent articles.

In addition, a need also exists for conductive elements for use in a wetness indicator that are made from non-metallic materials. Incorporating metallic components into an absorbent article, for instance, may cause various problems. For instance, once the absorbent articles are packaged, the absorbent articles are typically exposed to a metal detector to ensure that no metallic contaminants have accidentally been included in the package. Making the conductive elements of a wetness indicator from a metal, however, may cause a metal detector to indicate a false positive. The incorporation of metal conductive elements into an absorbent article may also cause problems when the wearer is attempting to pass through a security gate that also includes a metal detector.

### SUMMARY

The present disclosure is generally directed to a conductive nonwoven web that may be used in numerous applications. For example, in one embodiment, the nonwoven web may be used to form conductive elements of a wetness sensing device incorporated into an absorbent article. In one embodiment, the conductive nonwoven web contains a substantial amount of pulp fibers combined with conductive fibers and is formed

through a paper making process. The resulting web can then be easily incorporated into an absorbent article during its manufacture for forming an open circuit within the article. For example, in one embodiment, two strips or zones of the conductive nonwoven web are incorporated into an absorbent article for forming an open circuit. When a conductive substance extends between the two strips or conductive zones, a signaling device may be activated that produces a signal for indicating the presence of the conductive substance.

10 It should be understood that conductive webs made in accordance with the present disclosure may be used in numerous other applications in addition to being incorporated into a wetness sensing system for an absorbent article. For example, the conductive webs can be used in any suitable electronic device as a conductive element and/or as an antenna.

In one embodiment, the conductive nonwoven material comprises a nonwoven base web containing pulp fibers in an amount of at least about 50% by weight. Any suitable pulp fibers may be used. In one particular embodiment, for 15 instance, the pulp fibers comprise softwood fibers having a Canadian Standard Freeness (CSF) of at least about 350 mL. The softwood fibers can be present in the nonwoven base web in an amount of at least about 85% by weight.

In accordance with the present disclosure, the nonwoven 20 base web further includes conductive fibers, such as carbon fibers, that can be mixed with the pulp fibers. For example, in one embodiment, the carbon fibers are homogeneously mixed with the pulp fibers. The carbon fibers can be present in the base web in an amount from about 5% to about 15% by 25 weight. The carbon fibers can have a length of from about 1 mm to about 6 mm and can have a purity of at least about 85%, such as least about 88%. Purity refers to the amount of carbon contained in the carbon fibers.

The base web can have a basis weight of less than about 30 60 gsm, such as from about 15 gsm to about 40 gsm. The base web can also be uncreped and can have a tensile strength in the length direction of at least about 5900 gf. The base web can have a bulk of less than about 2 cc/g, such as less than about 1 cc/g. The base web can also have a resistance of less 35 than about 100 Ohms/square.

In one embodiment, the base web can include a wet 40 strength agent. The wet strength agent may comprise, for instance, a polyaminoamide-epichlorohydrin resin.

In one embodiment, the nonwoven material can be cut into 45 slits having a width of from about 3 mm to about 10 mm. The slits can be wound on a spool. For example, in one embodiment, the slits may be traverse wound on a spool.

The base web will generally have a gray or black color 50 depending upon the amount of carbon fibers contained in the web. In one embodiment, the base web can be dyed any suitable color. For instance, the web can be dyed a shade of blue or a shade of purple.

The present disclosure is also directed to a process for 55 producing a conductive paper web. The process includes the steps of depositing an aqueous suspension of fibers onto a porous forming surface to form a wet web. The aqueous suspension of fibers comprises softwood fibers mixed with carbon fibers. The carbon and softwood fibers can be as described above.

60 Once deposited onto the porous forming surface, the web can be flattened and then dried. The web can be flattened, for instance, by being fed through calendering rolls. The calendering rolls can apply a pressure of at least about 950 PLI. The web can be dried using any suitable drying device. For 65 instance, in one embodiment, the web can be placed adjacent to one or more drying cylinders that transfer heat to the web. Alternatively, the web can be through-air dried.

After being dried, the web can be slit into a plurality of slits having a width of from about 3 mm to about 10 mm. Each slit can be wound on a separate spool.

Other features and aspects of the present invention are discussed in greater detail below.

#### BRIEF DESCRIPTION OF THE DRAWINGS

A full and enabling disclosure of the present invention, including the best mode thereof to one of ordinary skill in the art, is set forth more particularly in the remainder of the specification, including reference to the accompanying figures in which:

FIG. 1 is a side view of one embodiment of a process for forming uncreped through-air dried webs in accordance with the present disclosure;

FIG. 2 is a side view of another embodiment of a process for forming conductive webs in accordance with the present disclosure;

FIG. 3 is a rear perspective view of one embodiment of an absorbent article made in accordance with the present disclosure;

FIG. 4 is a front perspective view of the absorbent article illustrated in FIG. 3;

FIG. 5 is a plan view of the absorbent article shown in FIG. 3 with the article in an unfastened, unfolded and laid flat condition showing the surface of the article that faces away from the wearer;

FIG. 6 is a plan view similar to FIG. 5 showing the surface of the absorbent article that faces the wearer when worn and with portions cut away to show underlying features;

FIG. 7 is a perspective view of the embodiment shown in FIG. 3 further including one embodiment of a signaling device;

FIG. 8 is a side view of still another embodiment of a process for forming conductive webs in accordance with the present disclosure;

FIG. 9 is a side view of one embodiment of a process for slitting a nonwoven material made in accordance with the present disclosure into a plurality of slits that are wound on individual spools; and

FIG. 10 is a side view of one embodiment of a spool that is used to wind the slits shown in FIG. 9.

Repeat use of reference characters in the present specification and drawings is intended to represent same or analogous features or elements of the present disclosure.

#### DETAILED DESCRIPTION

It is to be understood by one of ordinary skill in the art that the present disclosure is a description of exemplary embodiments only, and is not intended as limiting the broader aspects of the present disclosure.

In general, the present disclosure is generally directed to nonwoven webs containing conductive fibers. The conductive fibers can be incorporated into the web, for instance, such that the web is electrically conductive in at least one direction. For instance, the nonwoven web can be made so that it is capable of carrying an electric current in the length direction, in the width direction, or in any suitable direction.

In accordance with the present disclosure, the conductive nonwoven webs can contain a substantial amount of pulp fibers and can be made using a paper making process. For instance, in one embodiment, the conductive fibers can be combined with pulp fibers and water to form an aqueous suspension of fibers that is then deposited onto a porous surface for forming a conductive tissue web. The conductivity

of the tissue web can be controlled by selecting particular conductive fibers, locating the fibers at particular locations within the web and by controlling various other factors and variables. In one embodiment, for instance, the conductive fibers incorporated into the nonwoven web comprise chopped carbon fibers.

After a conductive nonwoven material is made in accordance with the present disclosure, the material can be cut into a plurality of slits that are then wound onto spools. Each slit, for instance, can have a width of from about 1 mm to about 15 mm, such as from about 3 mm to about 10 mm. Once wound onto a spool, each slit can be later incorporated into any suitable product.

Nonwoven webs made in accordance with the present disclosure may be used in numerous different applications. For instance, in one embodiment, the conductive nonwoven material may be incorporated into any suitable electronic device. For instance, the nonwoven web can be used as a fuel cell membrane, as a battery electrode, or may be used in printed electronics. For example, in one particular embodiment, the conductive fibers may form a patterned circuit within the base webs for any suitable end use application.

In one particular embodiment, the conductive nonwoven webs made in accordance with the present disclosure may be used to form wetness sensing devices within absorbent articles. The wetness sensing device, for instance, may be configured to emit a signal, such as an audible signal and/or a visible signal, when a conductive substance, such as urine or fecal matter, is detected in the absorbent article. In one embodiment, for instance, one or more nonwoven webs made in accordance with the present disclosure can be configured to form conductive elements within an absorbent article for creating an open circuit that is configured to close when a conductive substance is present in the article.

The absorbent article may be, for instance, a diaper, a training pant, an incontinence product, a feminine hygiene product, a medical garment, a bandage, and the like. Generally, the absorbent articles containing the open circuit are disposable meaning that they are designed to be discarded after a limited use rather than being laundered or otherwise restored for reuse.

The open circuit contained within the absorbent articles made from nonwoven webs of the present disclosure is configured to be attached to a signaling device. The signaling device can provide power to the open circuit while also including some type of audible and/or visible signal that indicates to the user the presence of a body fluid. Although the absorbent article itself is disposable, the signaling device may be reusable from article to article.

As described above, the base webs of the present disclosure are made by combining conductive fibers with pulp fibers to form nonwoven webs. In one embodiment, a tissue making process or a paper making process is used to form the webs.

The conductive fibers that may be used in accordance with the present disclosure can vary depending upon the particular application and the desired result. Conductive fibers that may be used to form the nonwoven webs include carbon fibers, metallic fibers, conductive polymeric fibers including fibers made from conductive polymers or polymeric fibers containing a conductive material, metal coated fibers, and mixtures thereof. Metallic fibers that may be used include, for instance, copper fibers, aluminum fibers, and the like. Polymeric fibers containing a conductive material include thermoplastic fibers coated with a conductive material or thermoplastic fibers impregnated or blended with a conductive material. For instance, in one embodiment, thermoplastic fibers may be used that are coated with silver.

The conductive fibers incorporated into the nonwoven material can have any suitable length and diameter. In one embodiment, for instance, the conductive fibers can have an aspect ratio of from about 100:1 to about 1,000:1.

The amount of conductive fibers contained in the nonwoven web can vary based on many different factors, such as the type of conductive fiber incorporated into the web and the ultimate end use of the web. The conductive fibers may be incorporated into the nonwoven web, for instance, in an amount from about 1% by weight to about 90% by weight, or even greater. In one embodiment, the conductive fibers can be present in the nonwoven web in an amount from about 5% by weight to about 15% by weight, such as from about 8% by weight to about 12% by weight.

Carbon fibers that may be used in the present disclosure include fibers made entirely from carbon or fibers containing carbon in amounts sufficient so that the fibers are electrically conductive. In one embodiment, for instance, carbon fibers may be used that are formed from a polyacrylonitrile (or PAN) polymer. In particular, the carbon fibers are formed by heating, oxidizing, and carbonizing polyacrylonitrile PAN polymer fibers. Such fibers typically have high purity and contain relatively high molecular weight molecules. For instance, the fibers can contain carbon in an amount greater than about 85% by weight. In one embodiment, for instance, the purity of the carbon fibers can be from about 85% to about 95%, such as from about 88% to about 92%. Although higher purity fibers have better conductive properties, the higher purity fibers can be more expensive. Sufficient electrical characteristics, on the other hand, can be obtained using fibers with the purity ranges described above.

In order to form carbon fibers from polyacrylonitrile PAN polymer fibers, the polyacrylonitrile PAN fibers are first heated in an oxygen environment, such as air. While heating, cyano sites within the polyacrylonitrile PAN polymer form repeat cyclic units of tetrahydropyridine. As heating continues, the polymer begins to oxidize. During oxidation, hydrogen is released causing carbon to form aromatic rings.

After oxidation, the fibers are then further heated in an oxygen starved environment. For instance, the fibers can be heated to a temperature of greater than about 1300° C., such as greater than 1400° C., such as from about 1300° C. to about 1800° C. During heating, the fibers undergo carbonization. During carbonization, adjacent polymer chains join together to form a lamellar, basal plane structure of nearly pure carbon.

Polyacrylonitrile-based carbon fibers are available from numerous commercial sources. For instance, such carbon fibers can be obtained from Toho Tenax America, Inc. of Rockwood, Tenn.

Other raw materials used to make carbon fibers are Rayon and petroleum pitch.

Of particular advantage, the formed carbon fibers can be chopped to any suitable length. In one embodiment of the present disclosure, for instance, chopped carbon fibers may be incorporated into the base web having a length of from about 1 mm to about 6 mm, such as from about 2 mm to about 5 mm. The fibers can have an average diameter of from about 3 microns to about 15 microns, such as from about 5 microns to about 10 microns. In one embodiment, for instance, the carbon fibers may have a length of about 3 mm and an average diameter of about 7 microns.

In one embodiment, the carbon fibers incorporated into the nonwoven base webs have a water soluble sizing. Sizing can be in the amount of 0.1-10% by weight. Water soluble sizings, can be, but not limited to, polyamide compounds, epoxy resin ester and polyvinyl pyrrolidone). In this manner, the sizing is dissolved when mixing the carbon fibers in water to provide a

good dispersion of carbon fibers in water prior to forming the nonwoven web. The sizing also assists in handling the fibers, by controlling them from becoming airborne while being added during the process.

5 In forming conductive nonwoven webs in accordance with the present disclosure, the above conductive fibers are combined with other fibers suitable for use in tissue or paper making processes. The fibers combined with the conductive fibers may comprise any natural or synthetic cellulosic fibers 10 including, but not limited to nonwoody fibers, such as cotton, abaca, kenaf, sabai grass, flax, esparto grass, straw, jute hemp, bagasse, milkweed floss fibers, algae fibers, and pineapple leaf fibers; and woody or pulp fibers such as those obtained from deciduous and coniferous trees, including softwood 15 fibers, such as northern and southern softwood kraft fibers; hardwood fibers, such as eucalyptus, maple, birch, and aspen. Pulp fibers can be prepared in high-yield or low-yield forms and can be pulped in any known method, including kraft, sulfite, high-yield pulping methods and other known pulping 20 methods. Fibers prepared from organosolv pulping methods can also be used, including the fibers and methods disclosed in U.S. Pat. No. 4,793,898, issued Dec. 27, 1988 to Laamanen et al.; U.S. Pat. No. 4,594,130, issued Jun. 10, 1986 to Chang et al.; and U.S. Pat. No. 3,585,104. Useful fibers can also be 25 produced by anthraquinone pulping, exemplified by U.S. Pat. No. 5,595,628 issued Jan. 21, 1997, to Gordon et al.

In one embodiment, softwood fibers are used to produce the nonwoven material. Softwood fibers tend to be longer which reduces particulate emission during manufacturing 30 and converting. The longer pulp fibers also have a tendency to entangle better with the conductive fibers, such as the carbon fibers.

The pulp fibers incorporated into the nonwoven material, 35 such as softwood fibers, can also be refined so as to increase the amount of bonding sites on each fiber. The increase in bonding sites increases the mechanical entanglement of the pulp fibers with the conductive fibers in the finished material. This allows for a very flat uniform paper with reduced carbon fiber fallout during processing. The refining action also 40 increases the overall strength of the nonwoven material. For example, in one embodiment, the pulp fibers can have a Canadian Standard Freeness of greater than about 350 mL, such as greater than about 375 mL. For instance, the pulp fibers can be refined so as to have a Canadian Standard Freeness of from about 350 mL to about 600 mL.

A portion of the fibers, such as up to 50% or less by dry 45 weight, or from about 5% to about 30% by dry weight, can be synthetic fibers such as rayon, polyolefin fibers, polyester fibers, polyvinyl alcohol fibers, bicomponent sheath-core fibers, multi-component binder fibers, and the like. An exemplary polyethylene fiber is Pulpex®, available from Hercules, Inc. (Wilmington, Del.). Synthetic cellulose fiber types include rayon in all its varieties and other fibers derived from viscose or chemically-modified cellulose.

55 Incorporating thermoplastic fibers into the nonwoven web may provide various advantages and benefits. For example, incorporating thermoplastic fibers into the web may allow the webs to be thermally bonded to adjacent structures. For instance, the webs may be thermally bonded to other nonwoven materials, such as a diaper liner which may comprise, for instance, a spunbond web or a meltblown web.

Chemically treated natural cellulosic fibers can also be used such as mercerized pulps, chemically stiffened or crosslinked fibers, or sulfonated fibers. For good mechanical 60 properties in using papermaking fibers, it can be desirable that the fibers be relatively undamaged and largely unrefined or only lightly refined. Mercerized fibers, regenerated cellulosic

fibers, cellulose produced by microbes, rayon, and other cellulosic material or cellulosic derivatives can be used. Suitable fibers can also include recycled fibers, virgin fibers, or mixtures thereof.

Other papermaking fibers that can be used in the present disclosure include paper broke or recycled fibers and high yield fibers. High yield pulp fibers are those papermaking fibers produced by pulping processes providing a yield of about 65% or greater, more specifically about 75% or greater, and still more specifically about 75% to about 95%. Yield is the resulting amount of processed fibers expressed as a percentage of the initial wood mass. Such pulping processes include bleached chemithermomechanical pulp (BCTMP), chemithermomechanical pulp (CTMP), pressure/pressure thermomechanical pulp (PTMP), thermomechanical pulp (TMP), thermomechanical chemical pulp (TMCP), high yield sulfite pulps, and high yield Kraft pulps, all of which leave the resulting fibers with high levels of lignin. High yield fibers are well known for their stiffness in both dry and wet states relative to typical chemically pulped fibers.

In general, any process capable of forming a tissue or paper web can be utilized in forming the conductive web. For example, a papermaking process of the present disclosure can utilize embossing, wet pressing, air pressing, through-air drying, uncreped through-air drying, hydroentangling, air laying, as well as other steps known in the art. The tissue web may be formed from a fiber furnish containing pulp fibers in an amount of at least 50% by weight, such as at least 60% by weight, such as at least 70% by weight, such as at least 85% by weight.

The nonwoven webs can also be pattern densified or imprinted, such as the tissue sheets disclosed in any of the following U.S. Pat. Nos. 4,514,345 issued on Apr. 30, 1985, to Johnson et al.; 4,528,239 issued on Jul. 9, 1985, to Trokhan; 5,098,522 issued on Mar. 24, 1992; 5,260,171 issued on Nov. 9, 1993, to Smurkoski et al.; 5,275,700 issued on Jan. 4, 1994, to Trokhan; 5,328,565 issued on Jul. 12, 1994, to Rasch et al.; 5,334,289 issued on Aug. 2, 1994, to Trokhan et al.; 5,431,786 issued on Jul. 11, 1995, to Rasch et al.; 5,496,624 issued on Mar. 5, 1996, to Steltjes, Jr. et al.; 5,500,277 issued on Mar. 19, 1996, to Trokhan et al.; 5,514,523 issued on May 7, 1996, to Trokhan et al.; 5,554,467 issued on Sep. 10, 1996, to Trokhan et al.; 5,566,724 issued on Oct. 22, 1996, to Trokhan et al.; 5,624,790 issued on Apr. 29, 1997, to Trokhan et al.; and, 5,628,876 issued on May 13, 1997, to Ayers et al., the disclosures of which are incorporated herein by reference to the extent that they are non-contradictory herewith. Such imprinted tissue sheets may have a network of densified regions that have been imprinted against a drum dryer by an imprinting fabric, and regions that are relatively less densified (e.g., "domes" in the tissue sheet) corresponding to deflection conduits in the imprinting fabric, wherein the tissue sheet superposed over the deflection conduits was deflected by an air pressure differential across the deflection conduit to form a lower-density pillow-like region or dome in the tissue sheet.

Wet and dry strength agents may be applied or incorporated into the base sheet. As used herein, "wet strength agents" refer to materials used to immobilize the bonds between fibers in the wet state. Typically, the means by which fibers are held together in paper and tissue products involve hydrogen bonds and sometimes combinations of hydrogen bonds and covalent and/or ionic bonds. In the present invention, it may be useful to provide a material that will allow bonding of fibers in such a way as to immobilize the fiber-to-fiber bond points and make them resistant to disruption in the wet state. In the present application, wet strength agents also assist in bonding the conductive fibers, such as the carbon fibers, to the rest of

the fibers contained in the web. In this manner, the conductive fibers are inhibited from falling out of the web during further handling.

Any material that when added to a tissue sheet or sheet results in providing the tissue sheet with a mean wet geometric tensile strength/dry geometric tensile strength ratio in excess of about 0.1 will, for purposes of the present invention, be termed a wet strength agent. Typically these materials are termed either as permanent wet strength agents or as "temporary" wet strength agents. For the purposes of differentiating permanent wet strength agents from temporary wet strength agents, the permanent wet strength agents will be defined as those resins which, when incorporated into paper or tissue products, will provide a paper or tissue product that 10 retains more than 50% of its original wet strength after exposure to water for a period of at least five minutes. Temporary wet strength agents are those which show 50% or less than, of their original wet strength after being saturated with water for 15 five minutes. Both classes of wet strength agents find application in the present invention. The amount of wet strength agent added to the pulp fibers may be at least about 0.1 dry weight percent, more specifically about 0.2 dry weight percent or greater, and still more specifically from about 0.1 to 20 about 3 dry weight percent, based on the dry weight of the 25 fibers.

Permanent wet strength agents will typically provide a more or less long-term wet resilience to the structure of a tissue sheet. In contrast, the temporary wet strength agents will typically provide tissue sheet structures that had low 30 density and high resilience, but would not provide a structure that had long-term resistance to exposure to water or body fluids.

The temporary wet strength agents may be cationic, non-ionic or anionic. Such compounds include PAREZ™ 631 NC 35 and PAREZ® 725 temporary wet strength resins that are cationic glyoxylated polyacrylamide available from Cytec Industries (West Paterson, N.J.). This and similar resins are described in U.S. Pat. No. 3,556,932, issued on Jan. 19, 1971, to Coscia et al. and U.S. Pat. No. 3,556,933, issued on Jan. 19, 40 1971, to Williams et al. Hercobond 1366, manufactured by Hercules, Inc., located at Wilmington, Del., is another commercially available cationic glyoxylated polyacrylamide that may be used in accordance with the present invention. Additional examples of temporary wet strength agents include 45 dialdehyde starches such as Cobond® 1000 from National Starch and Chemical Company and other aldehyde containing polymers such as those described in U.S. Pat. No. 6,224, 714, issued on May 1, 2001, to Schroeder et al.; U.S. Pat. No. 6,274,667, issued on Aug. 14, 2001, to Shannon et al.; U.S. 50 Pat. No. 6,287,418, issued on Sep. 11, 2001, to Schroeder et al.; and, U.S. Pat. No. 6,365,667, issued on Apr. 2, 2002, to Shannon et al., the disclosures of which are herein incorporated by reference to the extent they are non-contradictory herewith.

55 Permanent wet strength agents comprising cationic oligomeric or polymeric resins can be used in the present invention. Polyamide-polyamine-epichlorohydrin type resins also referred to as polyaminoamide-epichlorohydrin resins such as KYMENE 557H sold by Hercules, Inc., located at Wilmington, Del., are the most widely used permanent wet-strength agents and are suitable for use in the present invention. Such materials have been described in the following U.S. Pat. Nos. 3,700,623, issued on Oct. 24, 1972, to Keim; 3,772,076, issued on Nov. 13, 1973, to Keim; 3,855,158, 60 issued on Dec. 17, 1974, to Petrovich et al.; 3,899,388, issued on Aug. 12, 1975, to Petrovich et al.; 4,129,528, issued on Dec. 12, 1978, to Petrovich et al.; 4,147,586, issued on Apr. 3,

1979, to Petrovich et al.; and, 4,222,921, issued on Sep. 16, 1980, to van Eenam. Other cationic resins include polyethyl-enimine resins and aminoplast resins obtained by reaction of formaldehyde with melamine or urea. It can be advantageous to use both permanent and temporary wet strength resins in the manufacture of tissue products.

In one embodiment, a relatively large amount of a wet strength agent is incorporated into the nonwoven material. The wet strength agent may also add to the dry strength of the product. In addition, wet strength agents aid in the chemical entangling of the fibers in the material to improve the retention of the conductive fibers. The amount of wet strength agent added to the nonwoven material can depend upon various different factors. In general, for instance, the wet strength agent can be added in an amount from about 1 kg/mton to about 12 kg/mton, such as from about 5 kg/mton to about 10 kg/mton. In certain embodiments, it may be desirable to add as much wet strength agent as possible. In these embodiments, for instance, the wet strength agent can be added in amounts greater than about 7 kg/mton, such as in amounts greater than about 8 kg/mton.

Dry strength agents are well known in the art and include but are not limited to modified starches and other polysaccharides such as cationic, amphoteric, and anionic starches and guar and locust bean gums, modified polyacrylamides, carboxymethylcellulose, sugars, polyvinyl alcohol, chitosans, and the like. Such dry strength agents are typically added to a fiber slurry prior to tissue sheet formation or as part of the creping package.

Additional types of chemicals that may be added to the nonwoven web include, but is not limited to, absorbency aids usually in the form of cationic, anionic, or non-ionic surfactants, humectants and plasticizers such as low molecular weight polyethylene glycols and polyhydroxy compounds such as glycerin and propylene glycol. Materials that supply skin health benefits such as mineral oil, aloe extract, vitamin E, silicone, lotions in general and the like may also be incorporated into the finished products.

In general, the products of the present disclosure can be used in conjunction with any known materials and chemicals that are not antagonistic to its intended use. Examples of such materials include but are not limited to baby powder, baking soda, chelating agents, zeolites, perfumes or other odor-masking agents, cyclodextrin compounds, oxidizers, and the like. Of particular advantage, when carbon fibers are used as the conductive fibers, the carbon fibers also serve as odor absorbents. Superabsorbent particles, synthetic fibers, or films may also be employed. Additional options include dyes, optical brighteners, humectants, emollients, and the like.

Nonwoven webs made in accordance with the present disclosure can include a single homogeneous layer of fibers or may include a stratified or layered construction. For instance, the nonwoven web ply may include two or three layers of fibers. Each layer may have a different fiber composition. The particular fibers contained in each layer generally depends upon the product being formed and the desired results. In one embodiment, for instance, a middle layer contains pulp fibers in combination with the conductive fibers. The outer layers, on the other hand, can contain only pulp fibers, such as soft-wood fibers and/or hardwood fibers.

In one embodiment, nonwoven webs made in accordance with the present disclosure are generally made according to a wetlaid process. In this embodiment, the fibers are combined with water to form an aqueous suspension and then deposited onto a porous forming surface where a wet web is formed. In one embodiment, an aqueous suspension containing the pulp fibers is first produced. The conductive fibers, such as the

carbon fibers, are then injected into the aqueous suspension of pulp fibers prior to depositing the aqueous suspension onto the forming surface. For example, the conductive fibers can be injected into the aqueous suspension of pulp fibers in a headbox just prior to depositing the fibers onto the forming surface. The aqueous suspension of pulp fibers, for instance, may contain greater than 99% by weight water. For instance, in one embodiment, the aqueous suspension of pulp fibers contains the pulp fibers in an amount of less than 1% by weight, such as in an amount of about 0.5% by weight. The conductive fibers can then be injected into the aqueous suspension at a similar dilution. For instance, an aqueous suspension of carbon fibers containing carbon fibers in an amount of about 0.5% by weight may be injected into the aqueous suspension of pulp fibers.

Injecting the conductive fibers into an aqueous suspension of pulp fibers has been found to reduce the formation of flocks of the carbon fibers. It has been discovered that flocks have a greater tendency to form when the amount of time the fibers are mixed together increases. The creation of flocks, for instance, can produce weak spots in the resulting material and cause wet breaks when the nonwoven material is later processed.

Once the aqueous suspension of fibers is formed into a nonwoven web, the web may be processed using various techniques and methods. For example, referring to FIG. 1, shown is a method for making uncreped, throughdried tissue sheets. In one embodiment, it may be desirable to form the nonwoven web using an uncreped, through-air drying process. It was found that creping the nonwoven web during formation may cause damage to the conductive fibers by destroying the network of conductive fibers within the nonwoven web. Thus, the nonwoven web becomes non-conductive.

For simplicity, the various tensioning rolls schematically used to define the several fabric runs are shown, but not numbered. It will be appreciated that variations from the apparatus and method illustrated in FIG. 1 can be made without departing from the general process. Shown is a twin wire former having a papermaking headbox 34, such as a layered headbox, which injects or deposits a stream 36 of an aqueous suspension of papermaking fibers onto the forming fabric 38 positioned on a forming roll 39. The forming fabric serves to support and carry the newly-formed wet web downstream in the process as the web is partially dewatered to a consistency of about 10 dry weight percent. Additional dewatering of the wet web can be carried out, such as by vacuum suction, while the wet web is supported by the forming fabric.

The wet web is then transferred from the forming fabric to a transfer fabric 40. In one optional embodiment, the transfer fabric can be traveling at a slower speed than the forming fabric in order to impart increased stretch into the web. This is commonly referred to as a "rush" transfer. The relative speed difference between the two fabrics can be from 0-15 percent, more specifically from about 0-8 percent. Transfer is preferably carried out with the assistance of a vacuum shoe 42 such that the forming fabric and the transfer fabric simultaneously converge and diverge at the leading edge of the vacuum slot.

The web is then transferred from the transfer fabric to the throughdrying fabric 44 with the aid of a vacuum transfer roll 46 or a vacuum transfer shoe, optionally again using a fixed gap transfer as previously described. The throughdrying fabric can be traveling at about the same speed or a different speed relative to the transfer fabric. If desired, the through-drying fabric can be run at a slower speed to further enhance stretch. Transfer can be carried out with vacuum assistance to ensure deformation of the sheet to conform to the through-

## 11

drying fabric, thus yielding desired bulk and appearance if desired. Suitable throughdrying fabrics are described in U.S. Pat. No. 5,429,686 issued to Kai F. Chiu et al. and U.S. Pat. No. 5,672,248 to Wendt, et al. which are incorporated by reference.

In one embodiment, the throughdrying fabric provides a relatively smooth surface. Alternatively, the fabric can contain high and long impression knuckles.

The side of the web contacting the throughdrying fabric is typically referred to as the "fabric side" of the nonwoven web. The fabric side of the web, as described above, may have a shape that conforms to the surface of the throughdrying fabric after the fabric is dried in the throughdryer. The opposite side of the paper web, on the other hand, is typically referred to as the "air side". The air side of the web is typically smoother than the fabric side during normal throughdrying processes.

The level of vacuum used for the web transfers can be from about 3 to about 15 inches of mercury (75 to about 380 millimeters of mercury), preferably about 5 inches (125 millimeters) of mercury. The vacuum shoe (negative pressure) can be supplemented or replaced by the use of positive pressure from the opposite side of the web to blow the web onto the next fabric in addition to or as a replacement for sucking it onto the next fabric with vacuum. Also, a vacuum roll or rolls can be used to replace the vacuum shoe(s).

While supported by the throughdrying fabric, the web is finally dried to a consistency of about 94% or greater by the throughdryer 48 and thereafter transferred to a carrier fabric 50. The dried basesheet 52 is transported to the reel 54 using carrier fabric 50 and an optional carrier fabric 56. An optional pressurized turning roll 58 can be used to facilitate transfer of the web from carrier fabric 50 to fabric 56. Suitable carrier fabrics for this purpose are Albany International 84M or 94M and Asten 959 or 937, all of which are relatively smooth fabrics having a fine pattern. Although not shown, reel calendering or subsequent off-line calendering can be used to improve the smoothness and softness of the basesheet. Calendering the web may also cause the conductive fibers to orient in a certain plane or in a certain direction. For instance, in one embodiment, the web can be calendered in order to cause primarily all of the conductive fibers to lie in the X-Y plane and not in the Z direction. In this manner, the conductivity of the web can be improved while also improving the softness of the web.

In one embodiment, the nonwoven web 52 is a web which has been dried in a flat state. For instance, the web can be formed while the web is on a smooth throughdrying fabric. Processes for producing uncreped throughdried fabrics are, for instance, disclosed in U.S. Pat. No. 5,672,248 to Wendt, et al.; U.S. Pat. No. 5,656,132 to Farrington, et al.; U.S. Pat. No. 6,120,642 to Lindsay and Burazin; U.S. Pat. No. 6,096,169 to Hermans, et al.; U.S. Pat. No. 6,197,154 to Chen, et al.; and U.S. Pat. No. 6,143,135 to Hada, et al., all of which are herein incorporated by reference in their entireties.

In FIG. 1, a process is shown for producing uncreped through-air dried webs. It should be understood, however, that any suitable process or technique that does not use creping may be used to form the conductive nonwoven web. For example, referring to FIG. 2, another process that may be used to form nonwoven webs in accordance with the present disclosure is shown. In the embodiment illustrated in FIG. 2, the newly formed web is wet pressed during the process.

In this embodiment, a headbox 60 emits an aqueous suspension of fibers onto a forming fabric 62 which is supported and driven by a plurality of guide rolls 64. The headbox 60 may be similar to the headbox 34 shown in FIG. 1. In addition, the aqueous suspension of fibers may contain conductive

## 12

fibers as described above. A vacuum box 66 is disposed beneath forming fabric 62 and is adapted to remove water from the fiber furnish to assist in forming a web. From forming fabric 62, a formed web 68 is transferred to a second fabric 70, which may be either a wire or a felt. Fabric 70 is supported for movement around a continuous path by a plurality of guide rolls 72. Also included is a pick up roll 74 designed to facilitate transfer of web 68 from fabric 62 to fabric 70.

From fabric 70, web 68, in this embodiment, is transferred 10 to the surface of a rotatable heated dryer drum 76, such as a Yankee dryer. As shown, as web 68 is carried through a portion of the rotational path of the dryer surface, heat is imparted to the web causing most of the moisture contained within the web to be evaporated. The web 68 is then removed 15 from the dryer drum 76 without creping the web.

In order to remove the web 68 from the dryer drum 76, in one embodiment, a release agent may be applied to the surface of the dryer drum or to the side of the web that contacts the dryer drum. In general, any suitable release agent may be 20 used that facilitates removal of the web from the drum so as to avoid the necessity of creping the web.

Release agents that may be used include, for instance, polyamidoamine epichlorohydrin polymers, such as those sold under the trade name REZOSOL by the Hercules Chemical Company. Particular release agents that may be used in the present disclosure include Release Agent 247, Rezosol 1095, Crepetrol 874, Rezosol 974, ProSoft TQ-1003 all available from the Hercules Chemical Company, Busperse 2032, Busperse 2098, Busperse 2091, Buckman 699 all available from 30 Buckman Laboratories, and 640C release, 640D release, 64575 release, DVP4V005 release, DVP4V008 release all available from Nalco.

During the process of making the nonwoven material, such as either shown in FIG. 1 or FIG. 2, the web can be flattened 35 and densified. One technique for flattening or densifying the web is by feeding the web through the nip of opposing calender rolls. Flattening and densifying the sheet has been found to reduce fallout of the carbon fiber during further processing. Flattening the web reduces the overall caliper or 40 thickness and increases the electrical conductivity of the material by increasing the conductive fiber network and uniformity. Reducing the thickness of the material may also increase the run time of material rolls during product processing which improves efficiency, waste and delay. Increased conductivity may allow for an overall reduction in conductive fiber contained in the finished material.

When calendering the web, the web can be calendered in a dry state or in a wet state. In one embodiment, for instance, the calender rolls may apply a pressure of at least 900 PLI, such as from about 900 PLI to about 1100 PLI. For instance, in one particular embodiment, the pressure applied by the calendering rolls may be from about 950 PLI to about 1000 PLI, such as a pressure of about 980 PLI.

In an alternative embodiment, as shown in FIG. 8, the web 55 can be pressed against a plurality of drying cylinders that not only dry the web but flatten and densify the web. For example, referring to FIG. 8, a plurality of consecutive drying cylinders 80 are shown. In this embodiment, six consecutive drying cylinders are illustrated. It should be understood, however, 60 that in other embodiments more or less drying cylinders may be used. For example, in one embodiment, eight to twelve consecutive drying cylinders may be incorporated into the process.

As shown, a wet web 82 formed according to any suitable 65 process is pressed into engagement with the first drying cylinder 80. For example, in one embodiment, a fabric or suitable conveyor may be used to press the web against the surface of

the drying cylinder. The web is wrapped around the drying cylinder at least about 150°, such as at least about 180° prior to being pressed into engagement with the second drying cylinder. Each of the drying cylinders can be heated to an optimized temperature for drying the web during the process.

Nonwoven webs made in accordance with the present disclosure can have various different properties and characteristics depending upon the application in which the webs are to be used and the desired results. For instance, the nonwoven web can have a basis weight of from about 15 gsm to about 60 gsm or greater. In one embodiment, for instance, the new nonwoven web can have a basis weight of from about 30 gsm to about 40 gsm.

Once densified or flattened, the nonwoven web can be made with a relatively low bulk. For instance, as described above, in some processes, the web can be densified as it is formed. The bulk of these webs, for instance, may be less than about 2 cc/g, such as less than about 1 cc/g, such as less than about 0.5 cc/g.

The sheet "bulk" is calculated as the quotient of the caliper of a dry tissue sheet, expressed in microns, divided by the dry basis weight, expressed in grams per square meter. The resulting sheet bulk is expressed in cubic centimeters per gram. More specifically, the caliper is measured as the total thickness of a stack of ten representative sheets and dividing the total thickness of the stack by ten, where each sheet within the stack is placed with the same side up. Caliper is measured in accordance with TAPPI test method T411 om-89 "Thickness (caliper) of Paper, Paperboard, and Combined Board" with Note 3 for stacked sheets. The micrometer used for carrying out T411 om-89 is an Emveco 200-A Tissue Caliper Tester available from Emveco, Inc., Newberg, Oreg. The micrometer has a load of 2.00 kilo-Pascals (132 grams per square inch), a pressure foot area of 2500 square millimeters, a pressure foot diameter of 56.42 millimeters, a dwell time of 3 seconds and a lowering rate of 0.8 millimeters per second.

Nonwoven webs made in accordance with the present disclosure can also have sufficient strength so as to facilitate handling. For instance, in one embodiment, the webs can have a strength (or peak load) of greater than about 5000 grams force in the machine or length direction, such as greater than about 5500 grams force, such as even greater than about 6000 grams force. Tensile testing of the nonwoven material, for instance, can be conducted on a one inch wide specimen at 300 mm/min and 75 mm gage length.

The conductivity of the nonwoven web can also vary depending upon the type of conductive fibers incorporated into the web, the amount of conductive fibers incorporated into the web, and the manner in which the conductive fibers are positioned, concentrated or oriented in the web. In one embodiment, for instance, the nonwoven web can have a resistance of less than about 1500 Ohms/square, such as less than about 100 Ohms/square, such as less than about 80 Ohms/square. In one embodiment, for instance, the nonwoven material can have a resistance of from about 20 Ohms/square to about 80 Ohms/square, such as from about 20 Ohms/square to about 40 Ohms/square.

The conductivity of the sheet is calculated as the quotient of the resistive measurement of a sheet, expressed in Ohms, divided by the ratio of the length to the width of the sheet. The resulting resistance of the sheet is expressed in Ohms per square. More specifically, the resistance measurement is in accordance with ASTM F1896-98 "Test Method for Determining the Electrical Resistivity of a Printed Conductive Material". The resistance measuring device (or Ohm meter) used for carrying out ASTM F1896-98 is a Fluke multimeter

(model 189) equipped with Fluke alligator clips (model AC120); both are available from Fluke Corporation, Everett, Wash.

When using carbon fibers, the resulting nonwoven material is generally gray or black in color. If desired, the material may be dyed a particular shade of color to improve aesthetics. For instance, in one embodiment, the material can be dyed a shade of purple or a shade of blue. Particular dyes that may be used include PANTONE 264U purple dye or PANTONE 291 U blue dye.

10 The resulting conductive web made in accordance with the present disclosure may be used alone as a single ply product or can be combined with other webs or films to form a multiply product. In one embodiment, the conductive nonwoven web may be combined with other nonwoven webs to form a 15 2-ply product or a 3-ply product. The other nonwoven webs, for instance, may be made entirely from pulp fibers and can be made according to any of the processes described above.

In an alternative embodiment, the conductive nonwoven 20 web made according to the present disclosure may be laminated using an adhesive or otherwise to other nonwoven or polymeric film materials. For instance, in one embodiment, the conductive nonwoven web may be laminated to a meltblown web and/or a spunbond web that are made from polymeric fibers, such as polypropylene fibers. As described above, in one embodiment, the conductive nonwoven web can contain synthetic fibers. In this embodiment, the nonwoven web may be bonded to an opposing web containing synthetic fibers such as a meltblown web or spunbond web.

25 After the conductive nonwoven material of the present disclosure is formed, the material can be wound into a parent roll. The width of the formed material can vary depending upon the tissue or paper making process used. For instance, in general, the material can have a width of from about 60 inches to about 100 inches. In one embodiment, the nonwoven material is then cut into a plurality of slits for later use in various applications. For example, in one embodiment, the material can be slit to a width of from about 3 mm to about 12 mm, such as from about 5 mm to about 8 mm. In particular, the nonwoven material can be slit to a width to maintain strength and 30 electrical properties while minimizing raw material costs.

35 Since slitting of the material can produce conductive fiber fallout, in accordance with the present disclosure, the slitting can be performed in one step. For instance, one example of a slitting process in accordance with the present disclosure is shown in FIG. 9. The system illustrated in FIG. 9 is adapted to enclose and contain any free conductive fibers that may fall out from the material.

40 As shown in FIG. 9, a parent roll 84 comprised of the conductive nonwoven material 85 made according to the present disclosure is unwound into the process. In one embodiment, the parent roll 84 is center driven unwound so that no equipment is contacting the surface of the web. Surface driven unwind devices, on the other hand, can slip and 45 cause surface roughness and can cause inconsistent feed rates which may result in wet breaks.

45 From the parent roll 84, the nonwoven material 85 is first fed to a slitting device 86. The slitting device, for instance, may comprise a rotary slitter that slits the entire width of the nonwoven material simultaneously. The rotary slitter 86, for instance, may include rotary blades that are spaced apart a desired amount for forming the resulting slits.

50 As shown in FIG. 9, in one embodiment, after the material is cut, the resulting slits can be separated into a first group of slits 87 and a second group of slits 88. In one embodiment, for instance, the slits are divided in an alternative fashion in order to increase the spacing between the individual slits contained

## 15

in each group. Thus, one half of the slits can be fed overhead to form the first group of slits **87** while the other half of the slits can be fed below to form the second group of slits **88**.

The first group of slits **87** are then wound onto a first set of spools **89**, while the second group of slits **88** is wound on a second set of spools **90**. The first set of spools **89**, for instance, includes the spools **91**. The second set of spools **90**, on the other hand, includes the spools **92**. In the embodiment illustrated, each set of spools shows four individual spools. It should be understood, however, that more or less spools can be included in the system depending upon the number of slits that are produced.

As the group of slits **87** are fed downstream, each individual slit is then wound on a corresponding spool **91**. For example, a single slit **95** is shown being wound on the last spool **91**.

In order to be fed onto the spool, the slit is passed around a guide roll **96** and then fed to a tension control device **93**. The tension control device **93** maintains constant tension on the slit during the winding process. Due to the relatively high tensile strength of the material, for instance, small cross tensions on the web during converting and winding on the spools may cause the slits to break. Thus, in one embodiment, a tension control device can be associated with each slit for maintaining constant tension.

In one embodiment, for instance, the tension control device **93** may comprise a dancer roll that applies a force to the slit **95** for maintaining the slit under a constant and uniform tension.

As shown in FIG. 9, the slit **95** is wound onto the spool **91**. Once wound on the spool, the slit can be unwound into a separate process for the production of a particular article or product. In one embodiment, the slit can be traverse wound onto the spool **91**. Traverse winding takes the slit **95** and applies it to the spool core by traversing the length of the core. Traverse winding builds even and uniform rolls for later unwinding.

For example, referring to FIG. 10, the slit **95** is shown being wound onto the spool **91**. As shown in greater detail, the system can include a traversing arm **94** that moves back and forth in relation to the spool **91** as the slit **95** is wound on the spool.

As described above, nonwoven base webs made in accordance with the present disclosure may be used in numerous applications. For instance, the base webs may be used for their ability to conduct electric currents.

In one particular application, for instance, the conductive nonwoven web may be incorporated into a wetness sensing device that is configured to indicate the presence of a body fluid within an absorbent article. The wetness sensing device, for instance, may comprise an open circuit made from the conductive nonwoven material. The open circuit can be connected to a signaling device which is configured to emit an audible, visual or sensory signal when a conductive fluid closes the open circuit.

The particular targeted conductive fluid or body fluid may vary depending upon the particular type of absorbent article and the desired application. For instance, in one embodiment, the absorbent article comprises a diaper, a training pant, or the like and the wetness sensing device is configured to indicate the presence of urine. Alternatively, the wetness signaling device may be configured to indicate the presence of a metabolite that would indicate the presence of a diaper rash. For adult incontinence products and feminine hygiene products, on the other hand, the wetness signaling device may be configured to indicate the presence of a yeast or of a particular constituent in urine, such as a polysaccharide.

## 16

Referring to FIGS. 3 and 4, for exemplary purposes, an absorbent article **120** that may be made in accordance with the present invention is shown. The absorbent article **120** may or may not be disposable. It is understood that the present invention is suitable for use with various other absorbent articles intended for personal wear, including but not limited to diapers, training pants, swim pants, feminine hygiene products, incontinence products, medical garments, surgical pads and bandages, other personal care or health care garments, and the like without departing from the scope of the present invention.

By way of illustration only, various materials and methods for constructing absorbent articles such as the diaper **120** of the various aspects of the present invention are disclosed in 15 PCT Patent Application WO 00/37009 published Jun. 29, 2000 by A. Fletcher et al; U.S. Pat. No. 4,940,464 issued Jul. 10, 1990 to Van Gompel et al.; U.S. Pat. No. 5,766,389 issued Jun. 16, 1998 to Brandon et al., and U.S. Pat. No. 6,645,190 issued Nov. 11, 2003 to Olson et al. which are incorporated 20 herein by reference to the extent they are consistent (i.e., not in conflict) herewith.

A diaper **120** is representatively illustrated in FIG. 3 in a partially fastened condition. The diaper **120** shown in FIGS. 3 and 4 is also represented in FIGS. 5 and 6 in an opened and unfolded state. Specifically, FIG. 5 is a plan view illustrating the exterior side of the diaper **120**, while FIG. 6 illustrates the interior side of the diaper **120**. As shown in FIGS. 5 and 6, the diaper **120** defines a longitudinal direction **148** that extends from the front of the article when worn to the back of the article. Opposite to the longitudinal direction **148** is a lateral direction **149**.

The diaper **120** defines a pair of longitudinal end regions, otherwise referred to herein as a front region **122** and a back region **124**, and a center region, otherwise referred to herein 35 as a crotch region **126**, extending longitudinally between and interconnecting the front and back regions **122, 124**. The diaper **120** also defines an inner surface **128** adapted in use (e.g., positioned relative to the other components of the article **120**) to be disposed toward the wearer, and an outer surface **130** opposite the inner surface. The front and back regions **122, 124** are those portions of the diaper **120**, which when worn, wholly or partially cover or encircle the waist or mid-lower torso of the wearer. The crotch region **126** generally is that portion of the diaper **120** which, when worn, is positioned 40 between the legs of the wearer and covers the lower torso and crotch of the wearer. The absorbent article **120** has a pair of laterally opposite side edges **136** and a pair of longitudinally opposite waist edges, respectively designated front waist edge **138** and back waist edge **139**.

The illustrated diaper **120** includes a chassis **132** that, in this embodiment, encompasses the front region **122**, the back region **124**, and the crotch region **126**. Referring to FIGS. 3-6, the chassis **132** includes an outer cover **140** and a bodyside liner **142** (FIGS. 3 and 6) that may be joined to the outer cover **140** in a superimposed relation therewith by adhesives, ultrasonic bonds, thermal bonds or other conventional techniques. Referring to FIG. 6, the liner **142** may suitably be joined to the outer cover **140** along the perimeter of the chassis **132** to form a front waist seam **162** and a back waist seam **164**. As shown 50 in FIG. 6, the liner **142** may suitably be joined to the outer cover **140** to form a pair of side seams **161** in the front region **122** and the back region **124**. The liner **142** can be generally adapted, i.e., positioned relative to the other components of the article **120**, to be disposed toward the wearer's skin during 55 wear of the absorbent article. The chassis **132** may further include an absorbent structure **144** particularly shown in FIG. 6 disposed between the outer cover **140** and the bodyside liner **142**.

142 for absorbing liquid body exudates exuded by the wearer, and may further include a pair of containment flaps 146 secured to the bodyside liner 142 for inhibiting the lateral flow of body exudates.

The elasticized containment flaps 146 as shown in FIG. 6 define a partially unattached edge which assumes an upright configuration in at least the crotch region 126 of the diaper 120 to form a seal against the wearer's body. The containment flaps 146 can extend longitudinally along the entire length of the chassis 132 or may extend only partially along the length of the chassis. Suitable constructions and arrangements for the containment flaps 146 are generally well known to those skilled in the art and are described in U.S. Pat. No. 4,704,116 issued Nov. 3, 1987 to Enloe, which is incorporated herein by reference.

To further enhance containment and/or absorption of body exudates, the diaper 120 may also suitably include leg elastic members 158 (FIG. 6), as are known to those skilled in the art. The leg elastic members 158 can be operatively joined to the outer cover 140 and/or the bodyside liner 142 and positioned in the crotch region 126 of the absorbent article 120.

The leg elastic members 158 can be formed of any suitable elastic material. As is well known to those skilled in the art, suitable elastic materials include sheets, strands or ribbons of natural rubber, synthetic rubber, or thermoplastic elastomeric polymers. The elastic materials can be stretched and adhered to a substrate, adhered to a gathered substrate, or adhered to a substrate and then elasticized or shrunk, for example with the application of heat, such that elastic retractive forces are imparted to the substrate. In one particular aspect, for example, the leg elastic members 158 may include a plurality of dry-spun coalesced multifilament spandex elastomeric threads sold under the trade name LYCRA and available from Invista, Wilmington, Del., U.S.A.

In some embodiments, the absorbent article 120 may further include a surge management layer (not shown) which may be optionally located adjacent the absorbent structure 144 and attached to various components in the article 120 such as the absorbent structure 144 or the bodyside liner 142 by methods known in the art, such as by using an adhesive. A surge management layer helps to decelerate and diffuse surges or gushes of liquid that may be rapidly introduced into the absorbent structure of the article. Desirably, the surge management layer can rapidly accept and temporarily hold the liquid prior to releasing the liquid into the storage or retention portions of the absorbent structure. Examples of suitable surge management layers are described in U.S. Pat. No. 5,486,166; and U.S. Pat. No. 5,490,846. Other suitable surge management materials are described in U.S. Pat. No. 5,820,973. The entire disclosures of these patents are hereby incorporated by reference herein to the extent they are consistent (i.e., not in conflict) herewith.

As shown in FIGS. 3-6, the absorbent article 120 further includes a pair of opposing elastic side panels 134 that are attached to the back region of the chassis 132. As shown particularly in FIGS. 3 and 4, the side panels 134 may be stretched around the waist and/or hips of a wearer in order to secure the garment in place. As shown in FIGS. 5 and 6, the elastic side panels are attached to the chassis along a pair of opposing longitudinal edges 137. The side panels 134 may be attached or bonded to the chassis 132 using any suitable bonding technique. For instance, the side panels 134 may be joined to the chassis by adhesives, ultrasonic bonds, thermal bonds, or other conventional techniques.

In an alternative embodiment, the elastic side panels may also be integrally formed with the chassis 132. For instance, the side panels 134 may comprise an extension of the bodys-

ide liner 142, of the outer cover 140, or of both the bodyside liner 142 and the outer cover 140.

In the embodiments shown in the figures, the side panels 134 are connected to the back region of the absorbent article 120 and extend over the front region of the article when securing the article in place on a user. It should be understood, however, that the side panels 134 may alternatively be connected to the front region of the article 120 and extend over the back region when the article is donned.

With the absorbent article 120 in the fastened position as partially illustrated in FIGS. 3 and 4, the elastic side panels 134 may be connected by a fastening system 180 to define a 3-dimensional diaper configuration having a waist opening 150 and a pair of leg openings 152. The waist opening 150 of the article 120 is defined by the waist edges 138 and 139 which encircle the waist of the wearer.

In the embodiments shown in the figures, the side panels are releasably attachable to the front region 122 of the article 120 by the fastening system. It should be understood, however, that in other embodiments the side panels may be permanently joined to the chassis 132 at each end. The side panels may be permanently bonded together, for instance, when forming a training pant or absorbent swimwear.

The elastic side panels 134 each have a longitudinal outer edge 168, a leg end edge 170 disposed toward the longitudinal center of the diaper 120, and waist end edges 172 disposed toward a longitudinal end of the absorbent article. The leg end edges 170 of the absorbent article 120 may be suitably curved and/or angled relative to the lateral direction 149 to provide a better fit around the wearer's legs. However, it is understood that only one of the leg end edges 170 may be curved or angled, such as the leg end edge of the back region 124, or alternatively, neither of the leg end edges may be curved or angled, without departing from the scope of the present invention. As shown in FIG. 6, the outer edges 168 are generally parallel to the longitudinal direction 148 while the waist end edges 172 are generally parallel to the transverse axis 149. It should be understood, however, that in other embodiments the outer edges 168 and/or the waist edges 172 may be slanted or curved as desired. Ultimately, the side panels 134 are generally aligned with a waist region 190 of the chassis.

The fastening system 180 may include laterally opposite first fastening components 182 adapted for refastenable engagement to corresponding second fastening components 184. In the embodiment shown in the figures, the first fastening component 182 is located on the elastic side panels 134, while the second fastening component 184 is located on the front region 122 of the chassis 132. In one aspect, a front or outer surface of each of the fastening components 182, 184 includes a plurality of engaging elements. The engaging elements of the first fastening components 182 are adapted to repeatedly engage and disengage corresponding engaging elements of the second fastening components 184 to releasably secure the article 120 in its three-dimensional configuration.

The fastening components 182, 184 may be any refastenable fasteners suitable for absorbent articles, such as adhesive fasteners, cohesive fasteners, mechanical fasteners, or the like. In particular aspects the fastening components include mechanical fastening elements for improved performance. Suitable mechanical fastening elements can be provided by interlocking geometric shaped materials, such as hooks, loops, bulbs, mushrooms, arrowheads, balls on stems, male and female mating components, buckles, snaps, or the like.

In the illustrated aspect, the first fastening components 182 include hook fasteners and the second fastening components 184 include complementary loop fasteners. Alternatively, the

first fastening components **182** may include loop fasteners and the second fastening components **184** may be complementary hook fasteners. In another aspect, the fastening components **182, 184** can be interlocking similar surface fasteners, or adhesive and cohesive fastening elements such as an adhesive fastener and an adhesive-receptive landing zone or material; or the like. One skilled in the art will recognize that the shape, density and polymer composition of the hooks and loops may be selected to obtain the desired level of engagement between the fastening components **182, 184**. Suitable fastening systems are also disclosed in the previously incorporated PCT Patent Application WO 00/37009 published Jun. 29, 2000 by A. Fletcher et al. and the previously incorporated U.S. Pat. No. 6,645,190 issued Nov. 11, 2003 to Olson et al.

In the embodiment shown in the figures, the fastening components **182** are attached to the side panels **134** along the edges **168**. In this embodiment, the fastening components **182** are not elastic or extendable. In other embodiments, however, the fastening components may be integral with the side panels **134**. For example, the fastening components may be directly attached to the side panels **134** on a surface thereof.

In addition to possibly having elastic side panels, the absorbent article **120** may include various waist elastic members for providing elasticity around the waist opening. For example, as shown in the figures, the absorbent article **120** can include a front waist elastic member **154** and/or a back waist elastic member **156**.

As described above, the present disclosure is particularly directed to incorporating a body fluid indicating system, such as a wetness sensing device into the absorbent article **120**. In this regard, as shown in FIGS. 3-6, the absorbent article **120** includes a first conductive element **200** spaced from a second conductive element **202**. In this embodiment, the conductive elements extend from the front region **122** of the absorbent article to the back region **124** without intersecting. In accordance with the present disclosure, the conductive elements **200** and **202** can be made from a conductive nonwoven material as described above. In the embodiment illustrated in FIG. 4, the conductive elements **200** and **202** comprise separate and distinct strips or sheets. The strips, for instance, may comprise the slits shown in FIG. 9 that may have a width, for example, of from about 3 mm to about 12 mm.

The first conductive element **200** does not intersect the second conductive element **202** in order to form an open circuit that may be closed, for instance, when a conductive fluid is positioned in between the conductive elements. In other embodiments, however, the first conductive element **200** and the second conductive element **202** may be connected to a sensor within the chassis. The sensor may be used to sense changes in temperature or may be used to sense the presence of a particular substance, such as a metabolite.

In the embodiment shown in FIG. 3, the conductive elements **200** and **202** extend the entire length of the absorbent article **120**. It should be understood, however, that in other embodiments the conductive elements may extend only to the crotch region **126** or may extend to any particular place in the absorbent article where a body fluid is intended to be sensed.

The conductive elements **200** and **202** may be incorporated into the chassis **132** at any suitable location as long as the conductive elements are positioned so as to contact a body fluid that is absorbed by the absorbent article **120**. In this regard, the conductive elements **200** and **202** generally lie inside the outer cover **140**. In fact, in one embodiment, the conductive elements **200** and **202** may be attached or laminated to the inside surface of the outer cover **140** that faces the absorbent structure **144**. Alternatively, however, the conduc-

tive elements **200** and **202** may be positioned on the absorbent structure **144** or positioned on the liner **142**.

In order for the conductive elements **200** and **202** to be easily connected to a signaling device, the first conductive element **200** can include a first conductive pad member **204**, while the second conductive element **202** can include a second conductive pad member **206**. The pad members **204** and **206** are provided for making a reliable connection between the open circuit formed by the conductive elements and a signaling device that is intended to be installed on the chassis by the consumer.

The position of the conductive pad members **204** and **206** on the absorbent article **120** can vary depending upon where it is desired to mount the signaling device. For instance, in FIGS. 3, 5 and 6, the conductive pad members **204** and **206** are positioned in the front region **122** along the waist opening of the article. In FIG. 4, on the other hand, the conductive pad members **204** and **206** are positioned in the back region **24** along the waist opening of the article. It should be appreciated, however, that in other embodiments, the absorbent article **20** may include conductive pad members being positioned at each end of each conductive element **200** and **202**. In this manner, a user can determine whether or not to install the signaling device on the front or the back of the article. In still other embodiments, it should be understood that the pad members may be located along the side of the article or towards the crotch region of the article.

Referring to FIG. 7, for exemplary purposes, a signaling device **210** is shown attached to the conductive pad members **204** and **206**. The signaling device **210** includes a pair of opposing terminals that are electrically connected to the corresponding conductive pad members. When a body fluid is present in the absorbent article **120**, the open circuit formed by the conductive elements **200** and **202** is closed which, in turn, activates the signaling device **210**.

The signaling device **210** can emit any suitable signal in order to indicate to the user that the circuit has been closed.

## EXAMPLE

For exemplary purposes only, the following demonstrates the conductivity of base webs made in accordance with the present disclosure.

A conductive nonwoven web was made according to the present disclosure containing conductive carbon fibers. The conductive nonwoven web was made on a Fourdrinier 36" paper machine, which is located at the publicly accessible HERTY Advanced Materials Development Center located in Savannah, Ga.

A single layered web was produced containing a homogeneous blend of northern bleached softwood kraft fibers (LL19 from Terrace Bay Pulp Inc.), southern softwood kraft fibers (eucalyptus from Aracruz Celulose) and carbon fibers. The carbon fiber used was TENAX 150 fibers obtained from Toho Tenax having a cut length of 3 mm. The fiber furnish used to produce the web contained 94% by weight wood pulp fibers and 6% by weight carbon fibers. The wood pulp fiber blend contained 75% by weight softwood and 25% by weight hardwood.

The softwood furnish was refined using a 16" Beloit DD refiner with Finebar tackle to 365 CSF. The hardwood furnish was refined using 12" Sprout Twin Flow refiner to 365 CSF. Kymene 6500 from Hercules (Wilmington, Del.) was added to the furnish at 10 kilograms per metric ton of dry wood pulp fibers. The consistency of the stock fed to the headbox was about 2.43 weight %.

## 21

The formed conductive nonwoven web was also coated on both sides with starch PG280 from Penford Products (Cedar Rapids, Iowa) and latex CP620NA (a carboxylated styrene-butadiene latex) from Dow Chemical (Midland, Mich.) as shown in Table below.

In producing the samples, the wet formed web was contacted with a first set of dryer cans. After the first set of dryer cans, the web was fed through a size press and then contacted with a second set of dryer cans.

Process conditions for the samples were:

|                                           | Sample 1 | Sample 2 | Sample 3 |
|-------------------------------------------|----------|----------|----------|
| Machine Speed, FPM                        | 200      | 200      | 200      |
| Primary Thick Stock Flow, GPM             | 25       | 25       | 50       |
| Primary Total Flow, GPM                   | 200      | 200      | 200      |
| Holey Rolls, Direction                    | F        | F        | F        |
| Holey Rolls, RPM                          | 1800     | 1800     | 1800     |
| Primary H.B. Level, in.                   | 5        | 5        | 5        |
| Shake, %                                  | 90       | 90       | 90       |
| Vacuum, Inches of Water                   |          |          |          |
| Foil Box #1                               | 0        | 0        | 0        |
| #2                                        | 8        | 9        | 9        |
| #3                                        | 12       | 12       | 12       |
| #4                                        | 22       | 20       | 20       |
| #5                                        | 24       | 22       | 22       |
| Vacuum Flat Box No. 1 In. of Hg.          | 0        | 0        | 0        |
| No. 2                                     | 1        | 1        | 1        |
| No. 3                                     | 0        | 0        | 0        |
| Couch Roll, In. of Hg.                    | 9        | 6        | 6        |
| First Press, PLI                          | 280      | 280      | 280      |
| Second Press, PLI                         | 980      | 980      | 980      |
| First Dryer Section, Steam Pressure, PSI  | 8        | 8        | 8        |
| Size Press, PLI                           | —        | 36       | 36       |
| Pickup rate, lbs/Mton                     | —        | 140      | 140      |
| Second Dryer Section, Steam Pressure, PSI | 11       | 21       | 21       |

The resulting web was then tested for resistance. The following results were obtained:

|                                               | Sample 1 | Sample 2                   | Sample 3                                                  |
|-----------------------------------------------|----------|----------------------------|-----------------------------------------------------------|
| Coating at the size press                     | None     | 6 weight % add-on of PG280 | 10 weight % add-on of 50:50 mixture of PG2800 and CP620NA |
| Air dry basis weight (gsm)                    | 40       | 42                         | 42                                                        |
| Resistance (Ohms/square)                      | 70       | 80                         | 81                                                        |
| Bulk (cc/g)                                   | 2.1      | 2.2                        | 2.2                                                       |
| Machine direction tensile strength (grams/in) | 7892     | 10297                      | 10248                                                     |

The samples were tested for tensile strength using a tensile tester manufactured by MTS of Eden Prairie, Minn., equipped with TESTWORKS 3 software. The tester was set up with the following test conditions:

Gauge length=75 mm

Crosshead speed=300 mm/min.

Specimen width=1 inch (25.4 mm)

## 22

Peak load at break was recorded as the tensile strength of the material.

These and other modifications and variations to the present invention may be practiced by those of ordinary skill in the art, without departing from the spirit and scope of the present invention, which is more particularly set forth in the appended claims. In addition, it should be understood that aspects of the various embodiments may be interchanged both in whole or in part. Furthermore, those of ordinary skill in the art will appreciate that the foregoing description is by way of example only, and is not intended to limit the invention so further described in such appended claims.

What is claimed:

1. A process for producing a conductive paper web comprising:  
depositing an aqueous suspension of fibers onto a porous forming surface to form a wet web, the aqueous suspension of fibers comprising softwood fibers mixed with carbon fibers, the carbon fibers having a length of from about 1 mm to about 6 mm and having a purity of at least about 85%, the carbon fibers being present in an amount of from about 5% to about 15% based on the total weight of the fibers present; flattening the web; drying the web; slitting the web into a plurality of slits having a width of from about 3 mm to about 10 mm, each slit being wound on a separate spool, the slits being wound traversely on the spools.
2. A process as defined in claim 1, wherein the softwood fibers have a Canadian Standard Freeness of greater than about 350 mL.
3. A process as defined in claim 1, wherein the carbon fibers are coated with a water soluble size that is removed from the carbon fibers as the web is formed.
4. A process as defined in claim 1, wherein the carbon fibers have a purity of at least about 88%.
5. A process as defined in claim 1, wherein the slits have a final bulk of less than 1 g/cc.
6. A process as defined in claim 1, wherein the web is flattened by calendaring at a pressure of at least about 950 PLI.
7. A process as defined in claim 1, wherein an aqueous suspension of pulp fibers is formed first and then carbon fibers are injected into the aqueous suspension prior to depositing the fibers onto the forming surface.
8. A process as defined in claim 1, further comprising the step of incorporating a wet strength agent into the web.
9. A process as defined in claim 1, wherein the dried web is wound into a roll, the roll then being center driven unwound as the web is slit.
10. A process as defined in claim 9, wherein the plurality of slits are divided in an alternative fashion to from a first group of slits and a second group of slits, the first group of slits being fed to a first set of corresponding spools, the group of slits being fed to a second group of corresponding spools.
11. A process as defined in claim 1, wherein each spool is in association with a corresponding web tension device for controlling the tension of the slits as they are wound on the corresponding spools.
12. A process as defined in claim 11, wherein the tension device contains a dancer roll that is in communication with the slits as they are being wound on the spools, the process further including a traversing arm that directs the slits onto the spools for traversely winding the slits on the spools.

\* \* \* \* \*